# EUROPEAN PATENT SPECIFICATION

(11) **EP 0 152 455 B1**
(45) Date of publication and mention of the grant of the patent: **14.06.1989**
(21) Application number: 84903137.2
(22) Date of filing: 03.08.1984
(51) Int. Cl.: C10L 1/24

(54) **DIESEL FUEL AND METHOD FOR DEPOSIT CONTROL IN COMPRESSION IGNITION ENGINES**
DIESELBRENNSTOFF UND VERFAHREN ZUM STEUERN DES NIEDERSCHLAGS IN VERDICHTUNGSENTZÜNDUNGSMOTOREN
CARBURANT DIESEL ET PROCEDE POUR REGULER LE DEPOT DANS LE MOTEUR A ALLUMAGE PAR COMPRESSION

(30) Priority: 08.08.1983 US 521281; 30.09.1983 US 537894
(43) Date of publication of application: 28.08.1985
(73) Proprietor: CHEVRON RESEARCH AND TECHNOLOGY COMPANY, San Francisco, CA 94120 (US)
(72) Inventor: COURTNEY, Richard, L., San Rafael, CA 94901 (US)
(74) Representative: Kosmin, Gerald Emmanuel
(86) International application number: US8401243
(87) International publication number: WO8500827

(56) References cited:
- EP-A- 0 024 134
- EP-A- 0 100 665
- GB-A- 2 026 507
- US-A- 4 160 648
- US-A- 4 191 537
- US-A- 4 197 409
- US-A- 4 236 020
- US-A- 4 270 930
- US-A- 4 274 837
- US-A- 4 288 612
- US-A- 4 329 240

## Description

This invention relates to diesel engines, i.e. compression ignition internal combustion engines, and is concerned with the use of hydrocarbyl-terminated polyether polyamines as deposit control additives in diesel fuel in a concentration specifically designed to maintain or restore engine efficiency.

Until recently, in the United States, diesel engines were primarily limited to heavy uses such as trucks, farm equipment, and railroad engines. With the advent of the widespread acceptance of the passenger automobile utilizing a light-weight diesel engine, diesel fuels were required which did not give rise to severe noise and smoke problems such as those acceptable or tolerated in heavier engines.

Diesel fuels are susceptible to impurities which may arise from a variety of sources. They may occur in the fuel as produced or refined, or may through oxidation resulting from aging, produce soluble and insoluble materials of higher molecular weight and boiling point than the original fuel, which manifest themselves in the engine as colors or gums. Impurities may also be introduced in handling or from corrosion of storage vessels, either in the vehicle or in inventory. There may even be other additives specifically introduced by the manufacturer to solve or prevent some particular problem or improve the fuel itself, for example anti-oxidants, rust preventatives, and the like.

All of these impurities, however, may give rise to deposit formation in the fuel system of compression ignition engines, in particular, at the critical junctions of the fuel injectors. These deposits coat or adhere to injector parts and cause injector sticking, injector tip fuel metering passage fouling, nozzle hole plugging, leakage past critical surfaces, and delayed injection (and, hence, delayed start of combustion). These problems, in turn, result in significantly increased engine noise, smoke emissions, misfiring, low temperature or cold start problems, and idle roughness; and decreased power output and fuel economy.

It is believed that these engine problems are the result of long ignition delays, significantly contributed to by deposits, causing an excessively rapid pressure rise in the cylinder once combustion does occur. Recent evidence suggests that the long delay provides the time for certain chemical reactions to take place in the atomized fuel charge prior to ignition, resulting in products which burn exceedingly rapidly once combustion begins, thereby causing the undesirable rapid pressure rise, and the resultant problems. See "Gasoline and Other Motor Fuels Diesel Fuel", Encyclopedia of Chemical Technology, Kirk-Othmer, 3rd ed., Vol. 11, pp. 682-689.

It has been proposed to maintain the cleanliness of intake systems for spark-ignition internal combustion engines by incorporating in the gasoline fuel on which the engine operates a deposit control additive which is a hydrocarbyl-terminated polyoxyalkylene aminocarbamate in which a hydrocarbyl-terminated polyoxyalkylene component is linked to a polyamine component by a carbamate linkage, see for example our U.S. Patents Nos. 4191537 and 4270930.

According to one aspect of the present invention, deposit formation in the fuel system of compression ignition internal combustion engines is reduced by incorporating in the diesel fuel employed in the engine a deposit control additive which is a hydrocarbyl polyether polyamine having a molecular weight in the range from 500 to 2,500 and comprising a polyalkylene moiety containing from 1 to 30 oxyalkylene units each having from 2 to 4 carbon atoms which is bonded to a connecting moiety which in turn is bonded to an amino nitrogen atom of a polyamine moiety containing from 2 to 12 amine nitrogen atoms and from 2 to 40 carbon atoms, the hydrocarbyl polyether polyamine being present in the diesel fuel in a concentration of from 600 to 10,000 ppm.

According to another aspect of the invention, there is provided a method of reducing deposit formation in an internal combustion engine by incorporating in the hydrocarbonaceous fuel employed in said engine a deposit control additive, characterised in that the internal combustion engine is of the compression ignition type and the deposit control additive incorporated in the diesel fuel used in said engine is a hydrocarbyl polyether polyamine having a molecular weight in the range from 500 to 2,500 and comprising a polyalkylene moiety containing from 1 to 30 oxyalkylene units each having from 2 to 4 carbon atoms which is bonded to a connecting moiety which in turn is bonded to an amino nitrogen atom of a polyamine moiety containing from 2 to 12 amine nitrogen atoms and from 2 to 40 carbon atoms, the hydrocarbyl polyether polyamine being present in the diesel fuel in a concentration of from 600 to 10,000 ppm.

The method consists essentially of operating the engines using a fuel specifically designed for diesel or compression ignition engines and containing an effective amount of additive consisting of various polyether polyamines as defined above, preferably having a molecular weight of from 800 to 1500 which are soluble in hydrocarbon fuel boiling in the diesel fuel range. The boiling point of diesel fuel is ordinarily from 350°F (177°C) to 700°F (371°C). Alternatively, the method provides for introducing a concentrate containing the preferred additive into the fuel system of a compression ignition engine automobile to promote and maintain said cleanliness and efficiency. In either instance, using either an additized fuel or introducing a concentrate into the fuel; the method requires that the concentration of the additive must be sufficient to achieve in the desired effect. Generally, this concentration is from 600 to 10,000 ppm, and preferably from 1250 to 5,000 ppm.

The additives used to practice the method of the present invention are comprised of basically three moieties or components: a hydrophobic moiety at one end of the molecule comprising polyoxyalkylene polymer sub-moieties; a hydrophilic amine moiety at the other end; and a third moiety, a connecting group serving to unite the hydrophilic and hydrophobic ends of the molecule.

The polyoxyalkylene moiety comprises at least one oxyalkylene unit of from 2 to 4 carbon atoms and is terminated or "capped" with a hydrocarbyl group. The hydrocarbyl terminating group of the polyoxyalkylene moiety may contain from 1 to 30 carbon atoms. The polyoxyalkylene chain is bonded through a terminal oxygen to the appropriate connecting group which is in turn bonded to an amino nitrogen atom in the polyamine group. The polyamine contains from 2 to 12 amine nitrogens and from 2 to 40 carbon atoms, generally with a carbon-nitrogen ratio of between 1:1 and 10:1. The compounds have a molecular weight in the range from 500 to 2,500, and preferably from 800 to 1,500.

The additive consists of three parts or moieties. The first is the polyether or polyoxyalkylene moiety, which is hydrocarbyl terminated or "capped". The polyether moiety is bound through the second moiety, a connecting group or linkage to the nitrogen atom of the third moiety, the polyamine.

As fuel additives, the polyoxyalkylene moiety and the amine moiety are selected to provide solubility in the fuel, and clean-up properties within a diesel engine and its fuel system.

### Polyoxyalkylene moiety

The polyoxyalkylene moiety is ordinarily comprised of polyoxyalkylene polymers containing 1 to 30 oxyalkylene units, preferably 5 to 30 units, and more preferably 10 to 25 oxyalkylene units. When polymerized in the polymerization reaction, a single type of alkylene oxide may be employed. Copolymers, however, are equally satisfactory and random copolymers are readily prepared. Blocked copolymers of oxyalkylene units also provide satisfactory polyoxyalkylene polymers for the practice of the present invention.

The polyoxyalkylene moiety is terminated or "capped" by a hydrocarbyl terminating group. This terminating group may be comprised of an alkyl group of from 1 to 30 carbon atoms, an aryl group of from 6 to 30 carbon atoms, an alkaryl group of from 7 to 30 carbon atoms, an aralkyl group of from 7 to 30 carbon atoms, or a methylol - substituted alkyl group of from 5 to 30 carbon atoms.

The polyoxyalkylene moiety may ordinarily be prepared in a variety of ways, the most common for the practice of the present invention being by the reaction of an appropriate lower alkylene oxide containing from 2 to 4 carbon atoms with an appropriate initiator; for example, chlorohydrin or an alkyl phenol. In the preferred embodiment, dodecylphenol is used. Copolymers may be readily prepared by contacting the initiator compound with a mixture of alkylene oxides, while the blocked copolymers may be prepared by reacting the initiator first with one alkylene oxide and then another in any order or repetitively under polymerization conditions.

As an example, the polyoxyalkylene moiety derived from an alkyl - phenol - initiated polymerization detailed above is prepared as an alcohol containing a terminal hydroxyl group. The polyether moiety is then attached through the appropriate connecting group to the polyamine moiety by a variety of ways, preferably by reacting the hydroxyl group of the polyoxyalkylene unit with phosgene to form a polyoxyalkylene chloroformate and then reacting the polyoxyalkylene chloroformate with an amine. Alternatively, the hydroxyl group may be reacted with epichlorohydrin to give a methylol-substituted ethyl chloride end group. The resulting polyoxyalkylene alkyl chloride is then reacted with a polyamine to produce the composition of the present invention.

### The connecting group

The connecting group joining the polyoxyalkylene moiety with the amine moiety may be any relatively small diradical containing at least one carbon, oxygen, sulfur and/or nitrogen atom, and usually containing up to 12 carbon atoms. The connecting group which results and is used in the present composition is ordinarily a function of the method by which the compositions are formed and/or by which the components of the polyoxyalkylene moiety and the polyamine moiety are joined together.

Appropriate connecting groups include: methylol ethylene carbonyl and where Y and Y' independently=H, or an alkyl group of 1 or 2 carbon atoms.

### The amine moiety

The amine moiety of the polyether amine is derived from a polyamine having from 2 to 12 amine nitrogen atoms and from 2 to 40 carbon atoms. The polyamine preferably has a carbon to nitrogen ratio of from 1:1 to 10:1. The polyamine will contain at least 1 primary or secondary amine nitrogen atom. The polyamine may be substituted with a substituent group selected from (A) hydrogen; (B) hydrocarbyl groups from 1 to 10 carbon atoms; (C) acyl groups from 2 to 10 carbon atoms; and (D) monoketo, monohydroxy, monocyano, lower alkyl and lower alkoxy derivatives of (B), (C). "Lower", as used in lower alkyl and lower alkoxy, means a group containing 1 to 6 carbon atoms. "Hydrocarbyl" denotes an organic radical composed of carbon and hydrogen which may be aliphatic, alicyclic, aromatic or combinations thereof, e.g. aralkyl. The substituted polyamines employed in the present invention are generally, but not necessarily, N-substituted polyamines. The acyl groups falling within the definition of the aforementioned (C) substitutents are such as propionyl, acetyl, etc. The more preferred substituents are hydrogen, C₁ to C₆ alkyls, and Cₗ-C₆ hydroxyalkyls.

The more preferred polyamines finding use within the scope of the method of the present invention are polyalkylene polyamines, including alkylene diamine and substituted polyamines, e.g. alkyl and hydroxyalkyl - substituted polyalkylene polyamines. Preferably the alkylene groups contain from 2 to 6 carbon atoms, there being preferably 2 or 3 carbon atoms between the nitrogen atoms. Such groups are exemplified by ethyleneamines and include ethylene diamine, diethylene triamine, di(trimethylene) triamine, dipropylenetriamine, triethylenetetramine, etc. Such amines encompass isomers which are the branched-chain polyamines and the previously mentioned substituted polyamines, including hydroxy and hydrocarbyl - substituted polyamines. Among the polyalkylene polyamines, those containing 2 to 12 amine nitrogen atoms and 2 to 24 carbon atoms, are especially preferred and the C₂ to C₃ alkylene polyamines are most preferred, in particular, the lower polyalkylene polyamines, e.g. ethylene diamine, tetraethylenepentamine, etc.

In many instances a single compound will not be used as reactant in the preparation of the compositions used to practice this invention, in particular the polyamine component. That is, mixtures will be used in which one or two compounds will predominate with the average composition indicated.

A generalized, preferred formula for the polyether polyamines finding utility in this invention is as follows: wherein
R=an alkyl group of 1 to 30 carbon atoms, aryl group of 6 to 30 carbon atoms, alkaryl group of 7 to 30 carbon atoms, aralkyl group of 7 to 30 carbon atoms, or methylol-substituted alkyl group of 5 to 30 carbon atoms;
R' and R" independently=hydrogen, methyl or ethyl;
n=₁ to 30, preferably 10 to 25;
X=connecting group selected from the group consisting of: methylol ethylene carbonyl and where Y and Y' independently=H, or an alkyl group of 1 or 2 carbon atoms; and
Rⁱⁱⁱ=an amine moiety of the following general formula; wherein Z=the same or different constituent selected from:
   (I) hydrogen,
   (11) hydrocarbyl groups of 1 to 10 carbon atoms, and
   (III) hydrocarbonyl groups of 2 to 10 carbon atoms; and
Z₁=the same or different alkylene or hydroxy-substituted alkylene radical of 2 to 6 carbon atoms;
Z₂=carbonyl, alkylene carbonyl or alkylene of 2 to 4 carbon atoms with vicinal linkages; and
a=O or 1, preferably 1; b=0 to 4, preferably 0 to 2; c=₀ or 1, preferably 0; d=0 or 1, preferably 0; e=0 or 1, preferably 1; and f=0 or 1, and =1 when c=0, provided that b+2c+e+f equals at least 2.

The concentration of the additive which is necessary to achieve the desired deposit control effect is dependent upon a variety of factors, including the type of fuel used, the presence of other detergents or dispersants, or other additives, etc. Normally the range of concentration of the additive in the base fuel is from 600 to 10,000 weight ppm, preferably 1,000 to 6,000 weight ppm, and more preferably from 1,250 to 5,000 weight ppm of polyether polyamine.

The following examples are presented to illustrate a specific embodiment of the practice of this invention and should not be interpreted as a limitation upon the scope of that invention.

### Examples

### Example 1

In a general test of the clean-up ability of the method of the present invention, a West German-made automobile equipped with a diesel engine having the following history of injector problems and repairs was obtained:

At 34,382 miles (55,332 kilometers), a polybutene amine gasoline fuel detergent additive, distinctly different from the additive used in the present invention, was added to the diesel fuel to provide a concentration of 133 parts per million by weight of the additive in the diesel fuel. This polybutene gasoline fuel additive was added to the diesel fuel speculating that the injectors might be cleansed and the engine operation improved because of that additive's known ability to clean deposits from the carburetors of gasoline-fueled engines. Instead, the problems noted before recurred, i.e., rough running, excessive noise and smoke, and the automobile was hard to start.

At 38,753 miles (62,367 kilometers), the injectors were disassembled, inspected and photographed. All injectors had partially blocked central holes and deposits in the transverse bore.

The fouled test injectors were reinstalled and dodecylphenylpoly(oxybutylene) - N - (2 - aminoethyl) carbamate, an additive exemplary of that claimed for use in the present invention was added to a full fuel tank of automotive diesel fuel to a concentration of approximately 4,750 ppm active. A relatively immediate improvement in engine performance was noted, and after operation for 503 miles (809 kilometers) (i.e., through one tankful of additized fuel) the car was taken out of service and the injectors removed for inspection. It was observed that considerable deposits had been removed from the pintle central hole and the transverse bore.

### Example 2-injector clean-up

Six new diesel engine injector nozzles were tested for air flow at 0.1 mm pintle lift using the method of the International Standards Organization (ISO) number 4010-77. The values obtained are given in Table I in the column headed "New".

These injector nozzles were then installed in the diesel engine of a six-cylinder American-made diesel engine passenger car. This car was driven on a laboratory distance accumulator test stand under a program control that simulated city/suburban driving conditions. The average speed was 30 miles per hour (48 kilometers per hour). Regular commercial diesel fuel was used.

After about 1,026 miles (1,651 kilometers) the injector nozzles were removed and tested as described above. The results are shown in Table I. The injector nozzles were then reinstalled in the same engine and the distance accumulation continued. After a total of 2,256 miles (3,361 kilometers), the same measurements were made and are reported in Table I. At this time it was concluded that the deposits had stabilized.

The fuel was replaced by the same base diesel fuel, but now containing approximately 6,000 weight ppm of a 50% solution of dodecylphenylpoly(oxybutylene) - N - (2 - aminoethyl) carbamate in an inert, stable oleophilic organic solvent. The car was driven on the distance accumulator, under the same program control for an additional 375 miles (603 kilometers). The injector nozzles were removed and measured once again. The results are also given in Table I in the column headed "After Clean-up".

Examination of the data in Table I shows that after 1,026 miles (1,651 kilometers) of normal driving, the average air flow through the injectors, at 0.1 mm of pintle lift, is reduced from about 330 cm³/min. to about 110 cm³/min. An additional 1,230 miles (1,979 kilometers) of driving lowers this value to about 90 cm³/min. This decrease in airflow indicates a build-up of deposits in the injector nozzles limiting initial air flow to less than one-third the design amount. This reduction in the ISO test air flow relates directly to the reduction in diesel fuel quantity which will flow through such as nozzle, and in turn, this reduction in fuel flow causes hard starts, noise, emissions of unburned fuel, and other problems.

Surprisingly, the deposits in the fuel injectors are removed, and the flow rates returned to near normal by burning only about 13 gallons (49.2 liters) of fuel containing 3,000 weight ppm of an additive of the present invention. Additives that are effective at 0.1 mm of lift are also effective at other values of pintle lift (see Example 4).

### Example 3-Engine clean-up at various concentrations

Dirty injector nozzles were obtained from several different diesel engines of vehicles having combustion trouble as indicated by one or more of the following: noise, hard starts, exhaust smoke, low fuel economy, loss of power, rough idling, etc. These injector nozzles were installed in diesel vehicles which were then driven on a laboratory distance accumulator (see Example 2) until the air flow through the injector nozzles was about a constant value (ISO 4010-77) indicating stabilized deposits. The air flow rates at 0.1 mm pintle lift are given in Table II.

The diesel fuel was then additized with the indicated amount of dodecylphenylpoly(oxybutylene) - N - (2 - aminoethyl) carbamate, and the car was run under the same conditions as before until 20 gallons (75.7 liters) had been consumed (one tankful). The injector nozzles were again removed and the air flow rate measured. These values are given in Table II. After this measurement, the injector nozzles were manually cleaned by brushing to remove all deposits. Air flow rates were again measured, and are given in Table II.

(¹)Concentration of polyoxyalkylene polyamine additive.
⁽²⁾In some cases, not all of the engine injectors were on test because of a shortage of dirty injectors.

Percent clean-up, due to burning one tankful of diesel fuel containing an additive of the present invention, was calculated by setting the air flow after manual clean-up as 100% and the air flow just before changing to the test fuel as 0%. The calculated clean-up values based on this data suggests that the additive concentration necessary for injector nozzle clean-up is in the range of 600 to 10,000 ppm, preferably 1,000 to 6,000 ppm, and more preferably 1,500 to 5,000 ppm.

### Example 4-Cetane engine injector clean-up

The standard engine for determining cetane values by ASTM D 613-79 was fitted with a new Bosch injector nozzle, type DNO SD 240/. This engine stand was equipped with instruments for measuring: (1) combustion chamber pressure, (2) injector needle lift distance, and (3) crankshaft angle.

The engine was run at 900 RPM throughout the test. The compression ratio was adjusted to 21:1; the injection timing was set to 13° before top dead center and the amount of fuel injected was set at 13 ml/min. The cooling liquid was maintained at 212°F (100°C), the air intake at 150°F (66°C) and the oil temperature at 135°F (57°C). The fuel for this test was commercial #2 diesel (meeting ASTM D 975-78 specifications).

The air flow rate of the new nozzle was determined at several values of pintle lift by the method of ISO 4010-77. These values are given in Table III. The test engine was then run under the above described conditions for 20 hours. At the end of this time, the nozzle was removed and the air flow rate determined again. The results are given in Table III. The injector was reinstalled in the same engine which was then run for 20 additional hours with the same diesel fuel as before but now containing 10,000 ppm of a 50% solution of dodecylphenylpoly(oxybutylene) - N - (2 - aminoethyl) carbamate in an inert, stable oleophilic organic solvent. At the end of the second 20-hour run, the nozzle was removed and tested for air flow rate as before. The results are given in Table III.

The results in Table III show that running 20 hours on ordinary diesel fuel lays down sufficient deposits in a new injector nozzle to limit air flow to about 40 to 60% of its rate when new. After 20 hours of running on a diesel fuel containing an additive of the present invention, sufficient deposits in the injector nozzle are removed to restore the air flow to about 80 to 98% of the new nozzle rate.

## Claims

1. A fuel composition for use in an internal combustion engine comprising a hydrocarbonaceous liquid fuel containing a deposit control additive, characterised in that, in order for the fuel composition to be capable of use in an internal combustion engine of the compression ignition type, the liquid fuel is a hydrocarbon fuel boiling in the diesel fuel range and the deposit control additive is a hydrocarbyl polyether polyamine having a molecular weight in the range from 500 to 2,500 and comprising a polyalkylene moiety containing from 1 to 30 oxyalkylene units each having from 2 to 4 carbon atoms which is bonded to a connecting moiety which in turn is bonded to an amino nitrogen atom of a polyamine moiety containing from 2 to 12 amine nitrogen atoms and from 2 to 40 carbon atoms, the hydrocarbyl polyether polyamine being present in the diesel fuel in a concentration of from 600 to 10,000 ppm.

2. A fuel composition as claimed in Claim 1, wherein said connecting moiety contains up to 12 carbon atoms.

3. A fuel composition as claimed in Claim 1 or 2, wherein said polyoxyalkylene moiety comprises from 10 to 25 oxyalkylene units.

4. A fuel composition as claimed in Claim 1, 2 or 3, wherein said polyamine moiety contains from 2 to 12 amine nitrogen atoms and from 2 to 24 carbon atoms.

5. A fuel composition as claimed in Claim 1, wherein the deposit control additive is represented by the general formula: wherein
R=an alkyl group of 1 to 30 carbon atoms, aryl group of 6 to 30 carbon atoms, alkaryl group of 7 to 30 carbon atoms, aralkyl group of 7 to 30 carbon atoms, or methylol-substituted alkyl group of 5 to 30 carbon atoms;
Rⁱ and Rⁱⁱ independently=ₕydrogen, methyl or ethyl;
n=₁ to 30;
X=a connecting group selected from: methylol ethylene carbonyl and where Y and Y' independently=H, or an alkyl group of 1 or 2 carbon atoms; and
R"'=an amine moiety of the following general formula: wherein Z is the same or different substituent selected from:
(1) hydrogen,
(II) hydrocarbyl groups of 1 to 10 carbon atoms, and
(III) hydrocarbonyl groups of 2 to 10 carbon atoms;
Zᵢ=the same or different alkylene or hydroxy-substituted alkylene radical of 2 to 6 carbon atoms;
Z₂=carbonyl, alkylene carbonyl or alkylene of 2 to 4 carbon atoms with vicinal linkages; and
a=0 or 1;
b=0 to 4;
c=0 or 1;
d=0 or 1;
e=0 or 1; and
f=0 or 1, and =1 when c=0, provided that b+2c+e+f equals at least 2.

6. A fuel composition as claimed in Claim 1, wherein the additive is dodecylphenylpoly(oxybutylene) - N - (2 - aminoethyl)carbamate.

7. A method of reducing deposit formation in an internal combustion engine by incorporating in the hydrocarbonaceous fuel employed in said engine a deposit control additive, characterised in that the internal combustion engine is of the compression ignition type and the deposit control additive incorporated in the diesel fuel used in said engine is a hydrocarbyl polyether polyamine having a molecular weight in the range from 500 to 2,500 and comprising a polyalkylene moiety containing from 1 to 30 oxyalkylene units each having from 2 to 4 carbon atoms which is bonded to a connecting moiety which in turn is bonded to an amino nitrogen atom of a polyamine moiety containing from 2 to 12 amine nitrogen atoms and from 2 to 40 carbon atoms, the hydrocarbyl polyether polyamine being present in the diesel fuel in a concentration of from 600 to 10,000 ppm.

8. A method according to Claim 7, wherein the connecting moiety contains up to 12 carbon atoms.

9. A method according to Claim 7 or 8, wherein the polyoxyalkylene moiety comprises from 10 to 25 oxyalkylene units.

10. A method according to Claim 7, 8 or 9, wherein said polyamine moiety contains from 2 to 12 amine nitrogen atoms and from 2 to 24 carbon atoms.

11. A method according to Claim 7, wherein the deposit control additive is represented by the general formula: wherein
R=an alkyl group of 1 to 30 carbon atoms, aryl group of 6 to 30 carbon atoms, alkaryl group of 7 to 30 carbon atoms, aralkyl group of 7 to 30 carbon atoms, or methylol-substituted alkyl group of 5 to 30 carbon atoms;
R' and R" independently=hydrogen, methyl or ethyl;
n=1 to 30;
X=a connecting group selected from: methylol ethylene carbonyl and where Y and Y' independently=H, or an alkyl group of 1 or 2 carbon atoms; and
R"'=an amine moiety of the following general formula: wherein Z is the same or different substituent selected from:
(I) hydrogen, ^{I}
(II) hydrocarbyl groups of 1 to 10 carbon atoms, and
(III) hydrocarbonyl groups of 2 to 10 carbon atoms;
Z,=the same or different alkylene or hydroxy-substituted alkylene radical of 2 to 6 carbon atoms;
Z₂=carbonyl, alkylene carbonyl or alkylene of 2 to 4 carbon atoms with vicinal linkages; and
a=0 or 1;
b=0 to 4;
c=0 or 1;
d=0 or 1;
e=0 or 1; and
f=0 or 1, and =1 when c=0, provided that b+2c+e+f equals at least 2.

## Patentansprüche

1. Treibstoffzusammensetzung für eine Verwendung in einem Verbrennungsmotor aus einem kohlenwasserstoffartigen flüssigen Treibstoff, der ein Additiv für eine Ablagerungsbekämpfung enthält, dadurch gekennzeichnet, daß im Hinblick darauf, die Treibstoffzusammenzetung für eine Verwendung in einem Verbrennungsmotor des Diseltyps geeignet zu machen, der flüssige Treibstoff ein Kohlenwasserstofftreibstoff ist, der in dem Dieseltreibstoffbereich siedet, und das Additiv zur Ablagerungsbekämpfung ein Hydrocarbylpolyetherpolyamin mit einem Molekulargewicht im Bereich von 500 bis 2500 ist und einen Polyalkylenanteil, enthaltend 1 bis 30 Oxyalkyleneinheiten mit jeweils 2 bis 4 Kohlenstoffatomen, der mit einem verbindenden Anteil verbunden ist, aufweist, welcher seinerseits mit einem Aminostickstoffatom eines Polyaminanteils verbunden ist, der 2 bis 12 Aminostickstoffatome und 2 bis 40 Kohlenstoffatome enthält, wobei das Hydrocarbylpolyetherpolyamin in dem Dieseltreibstoff in einer Konzentration von 600 bis 10000 ppm vorliegt.

2. Treibstoffzusammensetzung nach Anspruch 1, wobei der verbindende Anteil bis zu 12 Kohlenstoffatome enthält.

3. Treibstoffzusammensetzung nach Anspruch 1 oder 2, wobei der Polyoxyalkylenanteil 10 bis 25 Oxyalkyleneinheiten aufweist.

4. Treibstoffzusammensetzung nach Anspruch 1, 2 oder 3, wobei der Polyaminanteil 2 bis 12 Aminstickstoffatome und 2 bis 24 Kohlenstoffatome enthält.

5. Treibstoffzusammensetzung nach Anspruch 1, wobei das Additiv zur Ablagerungsbekämpfung durch die allgemeine Formel wiedergegeben wird worin
R=eine Alkylgruppe mit 1 bis 30 Kohlenstoffatomen, Arylgruppe mit 6 bis 30 Kohlenstoffatomen, Alkarylgruppe mit 7 bis 30 Kohlenstoffatomen, Aralkylgruppe mit 7 bis 30 Kohlenstoffatomen oder Methylol - substituierte Alkylgruppe mit 5 bis 30 Kohlenstoffatomen
R' und R" unabhängig voneinander Wasserstoff,
Methyl oder Ethyl bedeuten,
n=1 bis 30,
X=eiₙe verbindende Gruppe, ausgewählt aus Methylolethylen 0 sowie wobei Y und Y' unabhängig voneinander für Wasserstoff oder eine Alkylgruppe mit 1 oder 2 Kohlenstoffatomen stehen und
Rⁱⁱⁱ=ein Aminoanteil der folgenden allgemeinen Formel worin Z ein gleicher oder verschiedener Substituent ist, ausgewählt aus
(I) Wasserstoff,
(11) Hydrocarbylgruppen mit 1 bis 10 Kohlenstoffatomen und
(III) Hydrocarbonylgruppen mit 2 bis 10 Kohlenstoffatomen,
Z₁=ein gleicher oder verschiedener Alkylen- oder Hydroxy - substituierter Alkylenrest mit 2 bis 6 Kohlenstoffatomen,
Z₂=Caᵣbonyl, Alkylencarbonyl oder Alkylen mit 2 bis 4 Kohlenstoffatomen mit benachbarten Verknüpfungen und
a=0 oder 1,
b=₀ bis 4,
c=0 oder 1,
d=0 oder 1,
e=0 oder 1 und
f=0 oder 1, und =1, wenn c=0, vorausgesetzt, daß b+2c+e+f wenigstens 2 ist.

6. Treibstoffzubereitung nach Anspruch 1, wobei das Additiv aus Dodecylphenylpoly(oxybutylen) - N - (2 - aminoethyl)carbamat besteht.

7. Verfahren zur Herabsetzung einer Ablagerungsbildung in einem Verbrennungsmotor durch Einbringen eines Additivs zur Ablagerungsbekämpfung in einen kohlenwasserstoffartigen Treibstoff, der in dem Motor verwendet wird, dadurch gekennzeichnet, daß der Verbrennungsmotor dem Dieseltyp entspricht und das in den Dieseltreibstoff, der in dem Motor verwendet wird, eingebrachte Additiv zur Ablagerungsbekämpfung ein Hydrocarbylpolyetherpolyamin mit einem Molekulargewicht im Bereich von 500 bis 2500 ist und einen Polyalkylenanteil, enthaltend 1 bis 30 Oxyalkyleneinheiten mit jeweils 2 bis 4 Kohlenstoffatomen, der wiederum mit einem Stickstoffatom eines Polyaminanteils, enthaltend 2 bis 12 Stickstoffatome und 2 bis 40 Kohlenstoffatome, verbunden ist, aufweist, wobei das Hydrocarbylpolyetherpolyamin in dem Dieseltreibstoff in einer Konzentration von 600 bis 10000 ppm vorliegt.

8. Verfahren nach Anspruch 7, wobei der verbindende Anteil bis zu 12 Kohlenstoffatome enthält.

9. Verfahren nach Anspruch 7 oder 8, wobei der Polyoxyalkylenanteil 10 bis 25 Oxyalkyleneinheiten aufweist.

10. Verfahren nach Anspruch 7,8 oder 9, wobei der Polyaminanteil 2 bis 12 Aminstickstoffatome und 2 bis 24 Kohlenstoffatome enthält.

11. Verfahren nach Anspruch 7, wobei das Additiv zur Ablagerungsbekämpfung der allgemeinen Formel entspricht, worin
R=eine Alkylgruppe mit 1 bis 30 Kohlenstoffatomen, Arylgruppe mit 6 bis 30 Kohlenstoffatomen, Alkarylgruppe mit 7 bis 30 Kohlenstoffatomen, Aralkylgruppe mit 7 bis 30 Kohlenstoffatomen oder Methylol - substituierte Alkylgruppe mit 5 bis 30 Kohlenstoffatomen
R' und R" unabhängig voneinander Wasserstoff, Methyl oder Ethyl bedeuten,
n=₁ bis 30,
X=eine verbindende Gruppe, ausgewählt aus Methylolethylen Carbonyl sowie wobei Y und Y' unabhängig voneinander für Wasserstoff oder eine Alkylgruppe mit 1 oder 2 Kohlenstoffatomen stehen und
R'"=ein Aminoanteil der folgenden allgemeinen Formel worin Z ein gleicher oder verschiedener Substituent ist, ausgewählt aus
(I) Wasserstoff,
(11) Hydrocarbylgruppen mit 1 bis 10 Kohlenstoffatomen und
(111) Hydrocarbonylgruppen mit 2 bis 10 Kohlenstoffatomen,
Z₁=ein gleicher oder verschiedener Alkylen- oder Hydroxy-substituierter Alkylenrest mit 2 bis 6 Kohlenstoffatomen,
Z₂=Carbonyl, Alkylencarbonyl oder Alkylen mit 2 bis 4 Kohlenstoffatomen mit benachbarten Verknüpfungen und
a=0 oder 1,
b=₀ bis 4,
c=0 oder 1,
d=0 oder 1,
e=0 oder 1 und
f=0 oder 1, und =1 wenn c=0, vorausgesetzt, daß b+2c+e+f wenigstens 2 ist.

## Revendications

1. Composition de carburant destinée à être utilisée dans un moteur à combustion interne, comprenant un carburant liquide hydrocarboné contenant un additif limitant les dépôts, caractérisée en ce que, afin que la composition de carburant soit capable d'être utilisée dans un moteur à combustion interne du type à allumage par compression, le carburant liquide est un carburant hydrocarboné bouillant dans la plage des carburants Diesel et l'additif limitant les dépôts est une hydrocarbylpolyéther - polyamine ayant un poids moléculaire de 500 à 2500 et comprenant un groupement polyalkylène contenant 1 à 30 motifs oxyalkylène, chacun renfermant 2 à 4 atomes de carbone, qui est lié à un groupe de jonction qui est à son tour lié à un atome d'azote de groupe amino d'un groupement polyamine content 2 à 12 atomes d'azote d'amine et 2 à 40 atomes de carbone, l'hydrocarbylpolyéther - polyamine étant présente dans le carburant Diesel en une concentration de 600 à 10 000 ppm.

2. Composition de carburant suivant la revendication 1, dans laquelle le groupe de jonction contient jusqu'à 12 atomes de carbone.

3. Composition de carburant suivant la revendication 1 ou 2, dans laquelle le groupement polyoxyalkylène comprend 10 à 25 motifs oxyalkylène.

4. Composition de carburant suivant la revendication 1, ou 3, dans laquelle le groupement polyamine contient 2 à 12 atomes d'azote d'amine et 2 à 24 atomes de carbone.

5. Composition de carburant suivant la revendication 1, dans laquelle l'additif limitant le dépôt est représenté par la formule générale: dans laquelle
R représente un groupe alkyle ayant 1 à 30 atomes de carbone, un groupe aryle ayant 6 à 30 atomes de carbone, un groupe alkaryle ayant 7 à 30 atomes de carbone, un groupe aralkyle ayant 7 à 30 atomes de carbone ou un groupe alkyle à substitution méthylol, ayant 5 à 30 atomes de carbone;
R' et R" représentent indépendamment l'hydrogène, un groupe méthyle ou éthyle;
n a une valeur de 1 à 30;
X représente un groupe de jonction choisi entre: méthyloléthylène carbonyle et -CHY-; où Y et Y' représentent indépendamment H ou un groupe alkyle ayant 1 ou 2 atomes de carbone; et
Rⁱⁱⁱ représente un groupement amine répondant à la formule générale suivante: dans laquelle les substituants Z représentent des substituants identiques ou différents choisis entre:
(1) l'hydrogène,
(II) des groupes hydrocarbyle ayant 1 à 10 atomes de carbone, et
(III) des groupes hydrocarbonyle ayant 2 à 10 atomes de carbone;
les radicaux Z₁ représentent des radicaux alkylène ou alkylène à substitution hydroxy, identiques ou différents, ayant 2 à 6 atomes de carbone;
les substituants Z₂ représentent des radicaux carbonyle, alkylènecarbonyle ou alkylène ayant 2 à 4 atomes de carbone avec les liaisons voisines; et
a a la valeur 0 ou 1;
b a une valeur de 0 à 4;
c a la valeur 0 ou 1;
d a la valeur 0 ou 1;
e a la valeur 0 ou 1; et
f a la valeur 0 ou 1 et est égal à 1 lorsque c est égal à 0, sous réserve que la somme b+2c+e+f soit au moins égale à 2.

6. Composition de carburant suivant la revendication 1, dans laquelle l'additif est le carbamate de dodécylphénylpoly(oxybutylène) - N - (2 - aminoéthyle).

7. Procédé pour réduire la formation de dépôts dans un moteur à combustion interne par incorporation au carburant hydrocarboné, utilisé dans ledit moteur, d'un additif limitant les dépôts, caractérisé en ce que le moteur à combustion interne est du type à allumage par compression et l'additif limitant les dépôts incorporé au carburant Diesel utilisé dans ledit moteur est une hydrocarbylpolyéther - polyamine ayant un poids moléculaire de 500 à 2500 et comprenant un groupement polyalkylène contenant 1 à 30 motifs oxyalkylène ayant chacun 2 à 4 atomes de carbone, qui est lié à un groupe de jonction qui est à son tour lié à un atome d'azote de groupe amino d'un groupement polyamine contenant 2 à 12 atomes d'azote d'amine et 2 à 40 atomes de carbone, l'hydrocarbylpolyéther - polyamine étant présente dans le carburant Diesel en une concentration de 600 à 10 000 ppm.

8. Procédé suivant la revendication 7, dans lequel le groupe de jonction contient jusqu'à 12 atomes de carbone.

9. Procédé suivant la revendication 7 ou 8, dans lequel le groupement polyoxyalkylène comprend 10 à 25 motifs oxyalkylène.

10. Procédé suivant la revendication 7, 8 ou 9, dans lequel le groupement polyamine contient 2 à 12 atomes d'azote d'amine et 2 à 24 atomes de carbone.

11. Procédé suivant la revendication 7, dans lequel l'additif limitant les dépôts est représenté par la formule générale: dans laquelle
R représente un groupe alkyle ayant 1 à 30 atomes de carbone, un groupe aryle ayant 6 à 30 atomes de - carbone, un groupe alkaryle ayant 7 à 30 atomes de carbone, un groupe aralkyle ayant 7 à 30 atomes de carbone ou un groupe alkyle à substitution méthylol, ayant 5 à 30 atomes de carbone;
R' et R" représentent indépendamment l'hydrogène, un groupe méthyle ou éthyle;
n a une valeur de 1 à 30;
X représente un groupe de jonction choisi entre: méthyloléthylène carbonyle et formules dans lesquelles Y et Y' représentent indépendamment H ou un groupe alkyle ayant 1 ou 2 atomes de carbone; et
R"' représente un groupement amine répondant à la formule générale suivante: dans laquelle les substituants Z représentent des substituants identiques ou différents choisis entre:
(I) l'hydrogène,
(II) des groupes hydrocarbyle ayant 1 à 10 atomes de carbone, et
(III) des groupes hydrocarbonyle ayant 2 à 10 atomes de carbone;
les radicaux Z₁ représentent des radicaux alkylène ou alkylène à substitution hydroxy, identiques ou différents, ayant 2 à 6 atomes de carbone;
les substituants Z₂ représentent des radicaux carbonyle, alkylènecarbonyle ou alkylène ayant 2 à 4 atomes de carbone avec les liaisons voisines; et
a a la valuer 0 ou 1;
b a une valeur de 0 à 4;
c à la valeur 0 ou 1;
d a la valeur 0 ou 1;
e a la valeur 0 ou 1; et
f a la valeur 0 ou 1 et est égal à 1 lorsque c est égal à 0, sous réserve que la somme b+2c+e+f soit au moins égale à 2.
